

Jan. 3, 1939.

L. A. HALL

2,142,871

HOMOGENEOUS ALKALINE DETERGENTS AND METHOD OF PRODUCING SAME

Filed June 14, 1937

FIG.1.

FIG.2.

FIG.3.

FIG.4.



Inventor:  
Lloyd A. Hall,  
By: Benjamin Almanza  
Attorney

## UNITED STATES PATENT OFFICE

2,142,871

HOMOGENEOUS ALKALINE DETERGENTS  
AND METHOD OF PRODUCING SAME

Lloyd A. Hall, Chicago, Ill., assignor to The Griffith Laboratories, Inc., a corporation of Illinois

Application June 14, 1937, Serial No. 148,018

12 Claims. (Cl. 87—5)

The present invention relates to improvements in alkaline compounds and more particularly in homogeneous alkaline detergents comprising or including phosphate compounds.

In the preparation and use of alkaline detergents and particularly those consisting partly or entirely of trisodium phosphate, difficulty has been encountered because, among other reasons, of the instability of such products in respect of their water content. Normal trisodium phosphate crystals have a very high water content, part of which is readily given up on changes in moisture content of the atmosphere and hence this material, as such, is uneconomical and produces dissatisfaction in use because of unsightliness, changes in condition of the material in opened packages and changes in its solubility, rate of solution, and strength with changes in water content. When prepared in the form of hydrates of lower water content or the anhydrous material, alone or in admixture with other alkalies, oxidizing agents and the like, the resulting products are likewise unstable, sometimes deliquescent and becoming wet in the package or causing reactions with other constituents of the detergent mixture; and sometimes causing caking or, on attempts to put the material in solution, agglomerating and forming masses which are not readily penetrated by the water and hence not readily dissolved. Attempts have been made to correct these difficulties by various expedients, among others by incorporating other alkaline detergents with the phosphate compounds; but in general these mixtures are unsatisfactory in character and performance, as they lack homogeneity and uniformity, or require special or elaborate technique in formation or crystallization; or if finely ground do not go into solution uniformly.

In accordance with the present invention, I am able to produce a borate-phosphate detergent of a completely homogeneous and uniform character, and which is economical and efficient, having a low water content, and is highly stable in respect of its water content. As a result, the product in accordance with the present invention, even when in finely powdered form, is in all respects uniform throughout in character and properties and may be permitted to remain in open packages without caking or becoming wet or unsightly, and may be employed in detergent mixtures, particularly with oxidizing agents, hypochlorites, perborates, and the like without causing reaction resulting from instability of water content.

In accordance with the present invention, trisodium phosphate and borax are dissolved partly or completely in water, and the resulting mixture heated for removal of water and to leave a minor proportion thereof, less than that required to satisfy the normal requirements of the constituents for water of crystallization and generally less than 25% and preferably in the range from 5 to 15%. The trisodium phosphate compound employed may be either anhydrous, the monohydrate, the normal crystalline dodecahydrate or some intermediate hydrated form. In carrying out the process for the production of the product according to the present invention, in the reduction of the water content of the solution or partial solution of the mixed constituents to a point below that required for the satisfaction of the normal hydration process in forming crystalline compounds of the constituent substances, a remarkable phenomenon occurs in that in the competition for water, there is apparently a complete dehydration of the phosphate constituent and, in fact, a tendency to convert the phosphate in the direction of the anhydrous pyro-compound, notwithstanding the presence of some proportions of water to the extent hereinbefore indicated, with the formation of a solid solution of the borate constituent in the phosphate constituent.

The change in structure of the constituents of the mixture as the result of the process of the present invention is clearly shown from an inspection of the characteristic X-ray diffraction patterns of the resulting products.

It is now well understood and established that such substances are distinguishable by the arrangement of the atoms and molecules making up the crystal and by the spacings between them; and that on passing an X-ray beam through the substance and permitting the diffracted beams to act on a photographic film or plate, a pattern is secured which is determined by the arrangement of the crystal lattice planes and which is characteristic of the substance. By passing a monochromatic beam of X-rays through a compacted powder mass of the substance and recording the diffracted rays upon a photographic emulsion surface, if the latter is disposed in the form of a cylindrical section with its axis perpendicular to the incident beam, the diffracted beams will be recorded as lines spaced from the position of the incident beam. The resulting patterns or traces are characteristic and their positions are determined by the spacings of the lattice planes of the definite crystalline substance or substances making up the molecules of the material under in-

vestigation ("Applied X-Rays" by George L. Clark, 2d ed., 1932, New York, pages 226 to 228 and 252, 253). Hydrated complexes, with water as a constituent part of the molecule, are thus distinguishable, as are solid solutions, in which the characteristic pattern of one of the constituents persists with but slight displacement of the positions of the lines due to the displacement of the lattice planes of the dominant constituent on intermolecular penetration of the other. The products of the present invention are shown by the similarity of the characteristic patterns to those of ignited anhydrous trisodium phosphate to be borate-phosphate compositions in which the borate constituent is present in the form of a solid solution in the anhydrous phosphate constituent. When these products are examined by X-ray analysis, their diffraction patterns show a substantial suppression or in some cases complete disappearance of the characteristic lines and spacings of borax, presenting those of anhydrous phosphates of the character resulting from the ignition of sodium phosphates with in some cases a slight displacement or doubling.

The invention will be more fully understood from the following description thereof, illustrated by the accompanying drawing, in which:

Figure 1 represents diagrammatically the characteristic X-ray diffraction pattern (recorded on a cylindrical film cassette) of anhydrous sodium phosphate ignited for 30 seconds:

Fig. 2 shows a characteristic pattern secured in a similar manner from a composition produced in accordance with the present invention; and

Figs. 3 and 4 show characteristic patterns produced in a similar manner from other products prepared in accordance with the present invention.

Referring more particularly to the drawing, as stated hereinbefore, Fig. 1 shows diagrammatically the principal lines and spacings of the characteristic pattern produced on a cylindrical film by diffraction of the K mono-chromatic X-ray beam from a copper anticathode by compacted powdered anhydrous sodium phosphate which has been ignited at white heat for 30 seconds. Certain of the stronger or more intense lines of the pattern have been indicated respectively by the numerals 1 to 16 inclusive.

In the drawing the representations of the characteristic patterns are diagrammatic, and the width and intensity of the lines being, however, indicated to the extent possible in such drawing.

Figs. 2, 3 and 4 represent diagrammatically characteristic patterns secured on X-ray analysis of products formed in accordance with the present invention, and will be described more fully in connection therewith.

In carrying out the present invention, the trisodium phosphate and borax in the desired proportions, with the constituents such as a sodium carbonate compound if desired, are mixed with water to form a slurry or to completely dissolve the mixture. The mixture may then be heated and agitated to effect partial or complete solution, and is then suitably heated to drive off water, leaving in the mixture less than sufficient water to satisfy the requirements of the constituents of the mixture for forming normally crystalline compounds, and preferably not more than 25%. The heating may be effected in open pans, driving off water until sputtering takes place, a temperature of 107 to 115° C. being reached, the mixture solidifying on cooling to a hard mass which may then, if desired, be heated at, say, 130-140° C.

to further reduce its moisture content, and may be ground to any desired degree of fineness; or it may be effected on a drum, for example, on chromium-plated drying drums at a temperature of 300 to 350° F.

The proportions of phosphate and borate constituents may vary considerably, the borate ranging from one-half to one-fourth of the solid constituents of the mixture. The phosphate constituent may be the normal crystalline trisodium phosphate, the monohydrate or the anhydrous compound. Varying proportions of a sodium carbonate compound such as sodium carbonate or sodium sesquicarbonate may be present, ranging up to 25 to 33% of the solid constituents of the mixture.

The following specific examples are illustrative:

3 parts by weight of monohydrated trisodium phosphate are mixed with 1 part by weight of borax and 2 parts by weight of water in one case and 4 parts in another, the admixture heated to effect partial or complete solution depending upon the proportion of water present, and evaporated to a water content of from 7 to 10%. In this product the molecular proportions are about 6.3 of phosphate to 1 of borax. The resulting products in the former case contained about 8.35% water and in the latter case about 7.35% water. These products gave identical characteristic X-ray diffraction patterns. In Fig. 2 is shown the characteristic diffraction pattern of these products secured under the conditions referred to in connection with the patterns of Fig. 1, previously described. The pattern does not show lines and spacings characteristic of borax. It does, however, show lines substantially similar in position and spacing to those of Fig. 1 with some slight variations and apparent omissions due to variations in intensity of lines in the record of the pattern, with but slight displacement, the respective lines being designated by the numerals 1b, 2b, 3b, 4b, 5b, 7b, 8b, 11b, and 13b and corresponding in position respectively with a slight displacement to the lines in the pattern of Fig. 1 bearing the same numbers but without the suffixes. An additional line 20b appears faintly on Fig. 2 that is not shown on Fig. 1, as but slight indication of its presence appears on the original record. It is to be noted, also, that the lines 11b, displaced somewhat with respect to the position of the line 11 of Fig. 1, are double in this pattern, and there is an inclination of doubling of the line 1b.

A product made in a similar manner by admixing 2 parts by weight of monohydrated trisodium phosphate, 1 part by weight of borax and 3 parts by weight of water, heating the mixture to effect solution and evaporating the resulting solution to about 5% water content, permitting the mass to solidify and grinding it to a powder, gave a product which recorded a characteristic X-ray diffraction pattern substantially identical with those previously referred to and illustrated in Fig. 2. In this product the molecular proportions are about 4.2 of phosphate to 1 of borax.

Using normal crystalline trisodium phosphate in varying proportions with borax and water to effect partial or complete solution and reducing the water content of the mixture to below 25% and preferably below 15%, the resulting product has a characteristic X-ray diffraction pattern illustrated in Fig. 3 which, it will be noted, is substantially similar in respect of most of the lines and their spacings to that of

Fig. 2. This same pattern has been produced with weight proportions of trisodium phosphate ranging from about 1 to about 3 times the proportion of borax initially present in the mixture. In this figure the lines 1c, 2c, 3c, 4c, 6c, 7c, 8c, 11c, 13c and 14c correspond in position to Fig. 1 bearing corresponding numbers (without the suffixes) in Fig. 1, and lines 11c and 20c to lines 11b and 20b of Fig. 2.

For example, 1 part of normal crystalline trisodium phosphate was mixed with 1 part of borax (or about equimolecular proportions) and 2 parts by weight of water, the mixture heated to effect solution and then heated in an open pan to remove water until the mixture had a low water content amounting to about 12.98% on the final product and congealed to a hard mass on cooling. The product was then powdered. By proceeding similarly with a mixture containing initially 3 parts of normal crystalline trisodium phosphate and 1 part of borax, with 4 parts of water, a product containing about 7.4% water was secured and each of these products, on X-ray analysis, gave the characteristic diffraction pattern shown in Fig. 3.

The compound produced as just described appears to be similar in so far as the nature of the phosphate constituent is concerned, to that which is produced with the monohydrated trisodium phosphate and borax when the former is in higher proportions than in the examples previously given. For example, when 1 part of monohydrated trisodium phosphate and 1 part by weight of borax with 2 parts by weight of water were heated to effect solution, and the solution dehydrated to about 12% water content, and the resulting mixture hardened on cooling, the powdered product gave, on X-ray analysis, a diffraction pattern substantially identical with that of Fig. 3.

The persistence of the numerous lines and their spacings in the patterns illustrated in Figs. 3 and 4 over the range of proportions of the constituents of the products yielding them clearly indicates their presence in the form of a solid solution in which the anhydrous phosphate constituent is present as the dominant constituent.

The presence of sodium carbonate or sodium sesquicarbonate in varying proportions up to 25 to 33% of the mixture does not appear to substantially alter the action which takes place. Thus, on mixing 2 parts of normal crystalline trisodium phosphate, 1 part of borax, 1 part of anhydrous sodium carbonate and 4 parts of water, heating the mixture to effect solution and subsequently evaporating the water from the mixture, a product was secured having a water content of about 12.7% and which, on X-ray analysis, failed to show distinctly either the characteristic patterns of borax or sodium carbonate, but did record a pattern as shown in Fig. 4, in which a number of the same characteristic lines and spacings are apparent as in Fig. 3, as indicated at 1d, 2d, 3d, 4d, 5d, 1d, 8d, 11d, 13d and 20d in Fig. 4, with additional less prominent lines probably due to the carbonate constituent. In this product the molecular proportions are about 2 of phosphate to 1 of borate to about 3.6 of carbonate. Substantially similar results were secured on using initially 1 part of monohydrated trisodium phosphate, 1 part of borax and 1 part of sodium carbonate with 3 parts of water; and also in another case by using 2 parts of normal trisodium phosphate, 1 part of borax, 1 part of sodium sesquicarbonate and 4 parts of water.

It will be apparent that the characteristic X-ray diffraction patterns of the products resulting from the carrying out of the present invention are strikingly similar to that of ignited trisodium phosphate as shown in Fig. 1. They do not have the characteristic lines and spacings of the pattern obtained from borax.

The borate-phosphate products of the present invention have been found to be markedly stable in respect of their water content. Even when finely powdered, they are completely uniform and homogeneous throughout and they do not tend to dry out excessively and likewise they do not tend to become wet, deliquesce, or cake. They dissolve readily and rapidly and do not tend to agglomerate and form difficultly soluble masses when poured or thrown into water to form solutions.

The products of the present invention are suitable for use as water softeners and are effective in improving the lathering qualities of soaps and the permanence of the lathers formed. They do not injuriously affect the hands and skin of users, as they are free from caustic alkali. They are excellent detergents or cleaners for use in dairies, bakeries, kitchens and the like, as they have but slight corrosive action upon tin and other metals (other than aluminum) commonly used therein. They are likewise excellent cleaners for stone, cement, metal work and the like.

By reason of the stability of their water content, the products of the present invention are also well adapted to form detergent mixtures or compositions with other substances, particularly those which are readily affected or decomposed by moisture and hence cannot ordinarily be used with phosphates, carbonates and other detergent alkalies which ordinarily yield a part of their moisture content readily or which tend to deliquesce or become wet in humid atmosphere.

Although the present invention has been described in connection with the details of specific examples embodying the same, it is not intended that these details shall be regarded as limitations on the scope of the invention, except in so far as included in the accompanying claims.

I claim:

1. The method of producing a homogeneous stable alkaline detergent product containing sodium borate and phosphate compounds in solid solution which comprises heating a trisodium phosphate and borax in the presence of a quantity of water greater than that in the final product and sufficient to form at least a slurry, the proportion of borax varying from about one-half to about one-fourth of the solid constituents, thereby driving off water and reducing the water content of the mixture to 5 to 25% thereof, whereby a stable solid solution is formed having an X-ray diffraction pattern including lines and spacings characteristic of ignited anhydrous sodium phosphate.

2. The method of producing a homogeneous stable alkaline detergent product containing sodium borate and phosphate compounds in solid solution which comprises heating a trisodium phosphate and borax in the presence of a quantity of water sufficient to dissolve the mixture, the proportion of borax varying from about one-half to about one-fourth of the solid constituents, thereby driving off water, and reducing the water content of the mixture to 5 to 25% thereof, thereby forming crystalline compounds, whereby a stable solid solution is formed having an X-ray diffraction pattern including lines and spacings

characteristic of ignited anhydrous sodium phosphate.

### 3. The method of producing a homogeneous.

stable alkaline detergent product containing sodium borate and phosphate compounds in solid solution which comprises heating a trisodium phosphate and borax in the presence of a quantity of water sufficient to at least form a slurry, the proportion of borax varying from about one-half to about one-fourth of the solid constituents, thereby driving off water and reducing the proportion of water to 5 to 15% of the mixture, whereby a stable solid solution is formed having an X-ray diffraction pattern including lines and spacings characteristic of ignited anhydrous sodium phosphate.

4. The method of producing a homogeneous stable alkaline detergent product containing sodium borate and phosphate compounds in solid solution which comprises heating a trisodium phosphate, borax and a sodium carbonate compound in the presence of a quantity of water sufficient to at least form a slurry, the proportion of borax varying from about one-half to about one-fourth of the solid constituents and the proportion of sodium carbonate compound being not in excess of about one-third of the solid constituents, thereby driving off water and reducing the water content of the mixture to 5 to 25% thereof, whereby a stable solid solution is formed having an X-ray diffraction pattern including lines and spacings characteristic of ignited anhydrous sodium phosphate.

5. The method of producing a homogeneous  
stable alkaline detergent product containing so-  
dium borate and phosphate compounds in solid  
solution which comprises heating a trisodium  
phosphate and borax in the presence of a quan-  
tity of water sufficient to at least form a slurry,  
the proportion of the trisodium phosphate be-  
ing from 1 to 3 times the proportion of the borax,  
thereby driving off water and reducing the wa-  
ter content of the mixture to 5 to 15% thereof,  
whereby a stable solid solution is formed hav-  
ing an X-ray diffraction pattern including lines  
and spacings characteristic of ignited anhydrous  
sodium phosphate.

50. 6. The method of producing a stable, alkaline detergent product containing sodium borate and phosphate compounds in solid solution which comprises heating a trisodium phosphate, a sodium carbonate compound and borax in the presence of a quantity of water sufficient to at least form a slurry, the proportion of said constituents being from 1 to 2 parts of the trisodium phosphate to 1 part of the borax and 1 part of the sodium carbonate compound, driving off water from the mixture and reducing the water content of the mixture to 5 to 15% thereof, whereby 55 a stable solid solution is formed having an X-ray diffraction pattern including lines and spacings characteristic of ignited anhydrous sodium phosphate.

7. A stable, homogeneous, alkaline borate-phosphate detergent product containing 5 to 15% of water and comprising in solid solution at least partly dehydrated crystalline compounds of trisodium phosphate and borax in which the

initial proportion of the phosphate compound is from 1 to 3 times that of the borax compound, and said product having an X-ray diffraction pattern including lines and spacings characteristic of ignited anhydrous sodium phosphate.

8. A stable, homogeneous, alkaline borate-phosphate detergent product containing water in proportions vary from about 5 up to 25% and comprising in solid solution at least partly dehydrated crystalline compounds of trisodium 10 phosphate and borax with sodium carbonate in which the carbonate is present in proportions not in excess of about one-third of the trisodium phosphate and borax and in which the initial proportion of the phosphate compound is from 15 1 to 3 times that of the borax compound, and said product having an X-ray diffraction pattern including lines and spacings characteristic of ignited anhydrous sodium phosphate.

9. A stable, homogeneous, alkaline borate-  
phosphate detergent product containing 5 to  
25% of water and comprising in solid solution  
at least partly dehydrated crystalline compounds  
of trisodium phosphate and borax in which the  
initial proportion of the phosphate compound is  
from 1 to 3 times that of the borax compound,  
the said product having an X-ray diffraction  
pattern including lines and spacings character-  
istic of ignited anhydrous sodium phosphate and  
being substantially free of lines characteristic of  
the borax compound. 30

10. A stable, homogeneous, alkaline borate-phosphate detergent product comprising in solid solution at least partly dehydrated crystalline compounds of trisodium phosphate and borax with sodium carbonate, the proportions of said constituents being from 1 to 3 parts of the trisodium phosphate compound to 1 part of the borax and 1 part of the sodium carbonate compound, said product containing in stable form 5 to 15% of water and having an X-ray diffraction pattern including lines and spacings characteristic of ignited anhydrous sodium phosphate. 35 40

11. A stable, homogeneous, alkaline borate-phosphate detergent comprising in solid solution at least partly dehydrated crystalline compounds of trisodium phosphate and borax in which the initial proportion of the phosphate compound is from 2 to 3 times that of the borax compound, the said product containing in stable form from 5 to 15% of water and having an X-ray diffraction pattern including lines and spacings characteristic of ignited anhydrous sodium phosphate. 43 50

12. A stable, homogeneous, alkaline detergent product containing water in proportions varying from 5 up to 25% and comprising in solid solution at least partly dehydrated crystalline compounds of trisodium phosphate and borax with sodium sesquicarbonate, the initial proportions of said constituents being from about 1 to 3 parts of the phosphate compound to 1 part of the borax and about 1 part of the carbonate compound, and having an X-ray diffraction pattern including lines and spacings characteristic of ignited anhydrous sodium phosphate. 55 60 65 70 75

LLOYD A. HALL